

July 23, 1946.

A. R. TRIST

2,404,606

# METHOD AND MACHINE FOR BURNISHING THE SURFACE OF PAPER

Filed Dec. 30, 1942

2 Sheets-Sheet 1



Arthur Ronald Trist  
INVENTOR

INVENTOR  
By Oldenbuck his ATT'y.

July 23, 1946.

A. R. TRIST

2,404,606

METHOD AND MACHINE FOR BURNISHING THE SURFACE OF PAPER

Filed Dec. 30, 1942

2 Sheets-Sheet 2



Fig. 2.



INVENTOR  
Arthur Ronald Trist  
By Oldenburt  
his ATT'y.

## UNITED STATES PATENT OFFICE

2,404,606

METHOD AND MACHINE FOR BURNISHING  
THE SURFACE OF PAPER

Arthur Ronald Trist, London W. 1, England

Application December 30, 1942, Serial No. 470,705  
In Great Britain February 21, 1942

8 Claims. (Cl. 92—68)

1

This invention relates to improvements in the treatment of the surface of paper to impart to said surface a desired "finish" in a convenient and economical manner.

The improved method of treatment produces by the simple means referred to, a similar result to that which is obtained by the use of the class of machine known generally as calenders, super calenders or friction glaziers and such like, which usually comprise highly polished chilled iron or steel rolls and paper bowls (in which the paper is highly compressed by hydraulic pressure) alternately arranged in a massive housing and requiring both skilled attention and considerable power, that is to say, the treatment imparts a "finish" to the surface operated on.

The invention contemplates passing the web to be treated between a resilient moving bed and one or more heated elastic blades trailing on and yieldingly co-operating with the web supported by said bed to "finish" the surface of said web that is contacted by the blade or blades.

The invention further contemplates the use of a suitably supported moving elastic bed, which may be an endless belt or a roller, the working surface in each case being composed of resilient material such as india rubber (natural or artificial) or any other substance capable of co-operating yieldingly with a trailing heated elastic blade or blades to impart the desired finish.

The invention also contemplates the use of one or more elastic blades made of a material which will not mark, that is to say, blacken, or impart other blemish to the web passing thereunder, such for example as steel, and so arranged that the edge trailing on the web can be heated in a regular and regulatable manner, for instance, by proximate thermostatically controlled electric heating coils or elements.

A simple machine for "finishing" paper webs may comprise a roller sheathed in india rubber, water cooled or not, and having one, two or more electrically heated elastic steel blades trailing thereon, the particular finish resulting from the passing of a web of paper between the outer surface of the roller (which travels with the web and supports it) and the blades, seemingly being dependent on the character of the paper web, the contact width of the blade or blades, the resilience of the sheathing on the roller, the degree of yielding co-operation between the edge or edges of the blade or blades and the web supported by the roller (bearing in mind that during operation the web itself co-operates with the india rubber sheathing and forms a factor in the resilience of

2

the bed at the point or points of operation), the angle of the blades to the surface of the roller, the temperature of the blades and the pressure of the contact edges of the blades on the web supported by the roller.

The actual values of the several factors can be determined only by experiment, but in some cases it may be necessary to laminate the steel blades and/or to modify the elasticity thereof by varying 5 the cross section by slots and/or apertures arranged so that the contact edge of such a blade is not interrupted.

Whether the webs treated are coated or not, the action of the machine consists in burnishing 10 the surface texture of the web to produce the required "finish" and gloss.

The invention can be carried into practice by many different mechanical constructions and therefore the arrangement described and shown 15 in the accompanying drawings must be regarded as by way of example only, and in order that the description may be understood reference will be had to the several figures of the drawings and to the letters marked thereon, like letters referring 20 to like or similar parts in the different figures in which:

Figure 1 is a sectional elevation showing diagrammatically the general arrangement of one 25 form of improved machine for finishing the surface of a web of paper;

Figure 2 is an end view of Figure 1 partly in section;

Figure 3 is a fragmentary detail of a modified form of blade;

Figure 4 is a cross section of Figure 3 taken on the line 4—4;

Figure 5 is a side elevation of a laminated blade;

Figure 6 is an exaggerated schematic view 40 showing the yielding co-operation between an elastic blade and a paper web supported by a resilient bed; and

Figure 7 is a fragmentary detail showing in general form the shape of the edge of a blade.

45 In the diagrammatic arrangement shown in Figures 1 and 2 the machine comprises a roller *a* journalled in side frames *b*, shown in chain lines in Figure 1, and rotated by a motor *c* so as to have a peripheral velocity of between, say, seven hundred and one thousand feet per minute.

The roller *a* is of comparatively large diameter, say between forty and fifty inches or so, and it has a thin wall *d* which is covered or clothed with a layer *e* of india rubber (natural or artificial) or 55 other resilient material having such physical

characteristics as will enable the peculiar effect described hereinafter to be obtained.

Usually it is found to be necessary to maintain the roller *a* cool and for this purpose, cold water, by way of example, is admitted through the pipe *f* to the sprays *gg* and is withdrawn through the pipe *h*, the pipes *f* and *h* passing through stuffing boxes or glands *i* in the trunnions of the roller *a*, but any other cooling arrangement may be used.

From Figure 1 it will be seen that the web *j* delivered from the supply roll travels in the direction of the arrow *k*, passes around the roller *a* and travels in the direction of the arrow *l* to the rewind mechanism.

The required "finish" is imparted to the external surface of the web *j* by means of one or more heated elastic blades *m* which trail on said surface at parts where the web *j* is supported by the resilient layer *e*.

In the simplest arrangement the blades *m* are made of spring steel or of a metal having a similarly high elastic limit and the composition of which does not include nickel, chromium or other ingredient which imparts or are likely to impart any blemish in the form of black marks or smudges, to the surface being treated.

Each blade *m* is clamped on a stock *n* which is pivotally mounted in the arms *o* carried by a shaft *p*, journaled in the side frames *b*, said shaft *p* having mounted thereon a lever *q* with a dead weight *r* on the end thereof or a mechanically equivalent spring arrangement.

The ends of the shafts *p* are threaded and each is provided with a lock nut *o*<sup>1</sup> and has a square *n*<sup>1</sup> so that the stock *n* can be angularly adjusted by applying keys to the squares *n*<sup>1</sup> and be clamped in adjusted position by tightening up the lock nuts *o*<sup>1</sup> thus enabling the angle of the blade *m* on the stock *n* to be set as may be desired.

The heating of the blades *m* is conveniently effected by thermostatically controlled electrical heaters *s* which, as shown, are located a short distance away from the under sides of the said blades, dissipation of heat from the exposed blade surface being reduced by means of the sheets *t* of asbestos cloth or the like.

The excellence and regularity of the "finish" obtained depends upon the careful correlation of the elasticity of the blade *m*, the angle of the blade *m* to the web *j*, the pressure per unit of area of the working face of the blade *m* the temperature of the blade *m* and the resilience of the paper covered layer *e* but does not seem to be very sensitive to changes in speed.

Each particular web surface requires special adjustment to obtain a particular "finish" and the following details will enable skilled overseers readily to obtain satisfactory results.

If the working face of the blade *m* is too wide, say sixty one thousandths of an inch or so, it flattens and irons a paper web without polishing it, and if the working face of the blade *m* is too thin, say ten one thousandths of an inch or so, it scrapes the surface and there is a tendency for the fibres to lift a little.

The temperature of the blade *m* may be between, say, three hundred and fifty and five hundred degrees of the Fahrenheit scale, the lower temperatures requiring greater pressure whilst the higher temperatures need less pressure.

The working face of the blade *m* is of great importance, it should be highly polished and shaped as shown at *m*<sup>1</sup> in Figure 7.

If the correct pressure is applied to a blade *m* at an appropriate angle to suit the elasticity of the

blade as well as the resilience of the paper covered layer *e*, the surface of the paper covered layer *e* will be very slightly indented so that a small ripple *e*<sup>1</sup> shown with gross exaggeration in Figure 6, forms behind and beneath the blade *m* thus causing the exposed surface of the web *j* to pass across the working face *m*<sup>1</sup> and experience a pressure which builds up from a minimum (zero) at the tip of the ripple, passes through a maximum at an intermediate zone on the working face and fades away to a minimum (zero) at the after edge of the depression continuously and smoothly from zero to zero.

When these conditions have been arranged by adjusting the angle of and selecting the thickness of the blade, adjustment of the temperature usually will produce any required "finish" that the paper is capable of taking.

As shown in the drawings the blade *m* is arranged at forty five degrees to a radius but this is by way of example only and may be varied within very wide limits to suit particular surface requirements.

The yielding co-operation between the elastic blades *m* and the resilient paper covered bed *e* is of great importance and in some cases that part of the blade *m* remote from the working face *m*<sup>1</sup> may have slots *m*<sup>2</sup> cut therein as shown in Figures 3 and 4 or the blade *m* carrying the working face *m*<sup>1</sup> may be reinforced by auxiliary blades *u* *v* and so on, to form a laminated structure as shown in Figure 5.

Usually it will be found that a single blade *m* is capable of producing any surface "finish" obtainable with a given paper web *j* regardless of the sizing used in the manufacture or the coating applied, but the invention is not limited to such single blade and in Figures 1 and 2 two blades are shown although it must be borne in mind that the effect due to the passage under the second blade may be quite different to the effect due to passage under the first blade so that the temperature, angle, elasticity, pressure and/or area of the working face of the second blade may be different to those of the first blade.

Practice has demonstrated that with certain papers there is an advantage in using more than one blade, but such practice also reveals that if too many blades are used the later blades destroy the "finish" produced by the earlier blades.

I claim:

1. In a method of burnishing the surface of paper, the steps of supporting a paper web to be burnished on a resilient bed and pressing a comparatively rigid blade having at its edge a thickness of more than 10 thousandths and less than 60 thousandths of an inch against said web at an oblique angle relative to the surface of the bed of sufficient magnitude to ensure contact between the web and the blade edge over the entire thickness of the latter and with sufficient force to depress a zone of said web corresponding substantially to the blade edge into said resilient bed while heating said blade and causing a relative movement of between about 700 and 1000 feet per minute between the surface of said resilient bed and web on the one hand and said blade on the other hand at substantially right angles to the edge of said blade and in such a way that the body of the blade overhangs the part of the web that is about to pass under the blade edge thereby forming directly adjacent said blade edge in said resilient bed a wave of resilient material, which presses a zone of said web adjacent said depressed

zone of said bed into frictional contact with a surface of said heated blade.

2. In a method of burnishing paper, the steps of supporting a web of paper to be burnished on a resilient moving bed and passing said web and bed at a surface speed of between about 700 and 1000 feet per minute beneath the more than 10 thousandths and less than 60 thousandths of an 10 ing thick edge of a trailing, stationary, comparatively rigid blade in a direction at substantially right angles to said edge and holding said blade at an oblique angle to the moving surface of a sufficient magnitude to ensure contact between said web and said blade edge over the entire thickness of the latter while heating said blade and pressing the edge thereof with sufficient force against said web to form an appreciable depression in said resilient bed beneath said edge and to create directly in the rear of said edge a wave 15 of resilient material the advancing front of which presses the surface of the web into frictional contact with the posterior surface of said heated blade.

3. A machine for burnishing paper comprising a resilient movable bed for supporting a paper 25 web to be burnished, means for advancing said bed in one direction at a surface speed of between about 700 and 1000 feet per minute, a resilient stationary blade having at its edge a thickness of more than 10 thousandths and less than 60 thousandths of an inch disposed at right angles to the direction of movement of said bed for trailing cooperation with its surface thereof at an oblique angle thereto of sufficient magnitude to ensure contact between a web supported on 30 said bed and the blade edge over the entire thickness of the latter, the relative resiliencies of said blade and bed being so chosen that upon pressure of the edge of said blade against a web supported on said bed the surface of the latter is deformed, means to press the edge of the blade against a web supported on said bed with sufficient force 35 to form an appreciable depression in the surface of said bed beneath said edge and to create directly in the rear of said edge a wave of resilient material the advancing front of which presses the surface of the web into frictional contact with the posterior surface of said blade, and means for heating said blade.

4. A machine, as claimed in claim 3, including means for cooling said resilient bed.

5. A machine, as claimed in claim 3, in which said blade has a curved surface portion leading from said edge to said posterior surface.

6. A machine, as claimed in claim 3, comprising at least one auxiliary blade disposed in contact with and cooperating with said trailing blade to augment the comparative rigidity of the latter, said auxiliary blade terminating short of the working edge of said trailing blade.

7. A machine for burnishing the surface of paper, comprising a resilient roller for supporting on its peripheral surface a web of paper to be burnished, side frames in which said roller is rotatably journaled, means for rotating said roller at a peripheral surface speed of between about 700 and 1000 feet per minute, a stationary, resilient, trailing blade having an edge of more than 10 thousandths and less than 60 thousandths of an inch and arranged parallel to the axis of said roller for cooperation with said peripheral surface, the relative resiliencies of said blade and roller being so chosen that upon pressure of the edge of said blade against a web supported on said roller the surface of the latter is deformed, a stock carrying said blade, said block being adjustably supported by said side frames to vary the position of said blade relative to the surface of said roller between various oblique angles each 30 of which is of sufficient magnitude to ensure contact between a web supported on said roller and the blade edge over the entire thickness of the latter, means for heating said blade, and means to press the edge of the blade against a web supported on the peripheral surface of the roller with sufficient force to form an appreciable depression in said peripheral surface beneath said edge and to create directly in the rear of said edge a wave of resilient material the advancing front of which presses the surface of the web into frictional contact with the heated posterior surface of said blade.

8. A machine, as claimed in claim 7, including means for water-cooling said resilient roller from the inside thereof.

ARTHUR RONALD TRIST.